

## UNITED STATES PATENT OFFICE

WILLIAM DALTON ROBINSON, OF CHERRYVILLE, NORTH CAROLINA

## COATING FOR COTTON MILL ROLLS

No Drawing.

Application filed February 27, 1929. Serial No. 343,245.

The invention relates to a coating material adapted to be applied to leather rollers in cotton mills, and has for its object to provide a coating material, which will preserve the 5 rollers and prevent the cracking of the leather.

A further object is to provide a leather coating and preservative for cotton mill rollers comprising a mixture of dry red lead, 10 oil of origanum, lamp black, glycerine, French gelatine and acetic acid. The proportions of the ingredients are preferably two and one half ounces of red lead; two and one half ounces of origanum, two ounces of 15 lamp black; two and one half ounces of glycerine; one and one half pounds of French gelatine, and to which is added sufficient acetic acid to make one gallon of liquid material.

20 In carrying out the invention, the dry red lead and lamp black are mixed with the liquid ingredients and thoroughly stirred; then the glycerine and gelatine are added to the combination of ingredients, which will dissolve 25 the gelatine.

It has been found that a coating material formed from the above ingredients when applied to leather rollers will positively preserve the rollers and prevent cracking or deterioration thereof. It has also been found 30 that the material can be cheaply manufactured and sold, and will not deteriorate with age or separate.

The acetic acid acts as a solvent for the 35 glycerine and holds it in solution, thereby making a compound which adheres to the rollers. The oil of origanum is placed in the solution as a drying agent, and the glycerine adds life to the compound and prevents 40 cracking of the coating. The red lead and lamp black are suspended in the compound and adds toughness thereto so that the strands of cotton will roll on and off the rollers, and to add color, for instance the lamp 45 black, which also acts as a filler and to aid lead in making grainy surface on rollers.

The invention having been set forth what is claimed as new and useful is:—

50 A leather coating material comprising a mixture of two and one half ounces of dry

red lead, two and one half ounces oil of origanum, two ounces of lamp black, two and one half ounces of glycerine, one and one half pounds of gelatine and sufficient acetic acid to make one gallon.

55

In testimony whereof he hereunto affixes his signature.

WILLIAM DALTON ROBINSON.

60

65

70

75

80

85

90

95

100